

## UNITED STATES PATENT OFFICE

J BIRCHARD GREEN, OF CHICAGO, ILLINOIS, ASSIGNOR TO CHICAGO STEEL AND WIRE COMPANY, OF CHICAGO, ILLINOIS, A CORPORATION OF ILLINOIS

## METHOD OF MAKING CEMENT-COATED WIRE

No Drawing.

Application filed November 23, 1927. Serial No. 235,402.

The object of my invention is to apply a film or layer of cementing material to a metallic wire or strip in such a manner that the coating is smooth, flexible, hard and suitable for use in an automatic forming machine without serious interference with the operation of such machine, said coating increasing the holding power of fastening devices made from the wire when driven into wood or like materials.

My invention relates to the application of such a coating to continuous lengths or coils of wire, in distinction to wire after it has been formed into various articles, such as staples, 15 nails, and the like. I have found that there are only a few methods by which this can be done satisfactorily. One method, for example, is to draw the wire through a solution or dip. Another is to spray the coating 20 material onto the wire, either as a single strand or in the coil. Still another is to dip the coil in the solution. While these represent the fundamental methods, the details 25 may differ. For instance, the material may be applied hot or cold; it may be a solution at ordinary temperatures; or it may be a material which must be fused in order to make it liquid, etc.

I prefer to dip the wire in coils because 30 less equipment is required, the equipment necessary is quite inexpensive, and the process is altogether simpler and cheaper to perform as a manufacturing operation. However, when the wire is dipped as a coil in any 35 cementing material, the material, being gummy, will naturally cause the various strands to adhere together and prevent a smooth coating being formed. I have discovered that I can overcome this by spreading the coil of wire out on a mandrel which 40 is of substantially less diameter than the inside diameter of the coil of wire, and rotating the mandrel during the drying of the coating material, whereby a shifting contact 45 between the supporting mandrel and the wire is obtained. Immediately after dipping the coil, the coating material is quite liquid, and as this coating material dries, or solidifies, it changes gradually from a liquid 50 to a solid. While the coating material is

quite liquid, every contact between adjacent strands of wire and also every contact with the supporting mandrel disturbs or roughens the coating. I have found, however, that the moment the point of contact, either between 55 adjacent strands or with the supporting mandrel, is shifted, the coating material tends to spread out again over the surface of the wire and heals the roughened spot. By the time the same point on the wire makes another 60 contact, the coating material is more nearly solid and the contact does not roughen it quite so much. On the other hand, it has a slower tendency to heal but I have discovered that these two tendencies may be made to balance out in such a way that the tendency to 65 heal the roughened spots is greater than the tendency to produce such spots.

The result is that when the coating material is dried or solidified, the wire is smoothly and evenly coated. I have found that the tendency toward a smooth coating, when the wire is dipped as a coil and the coating material dried or solidified on a shifting contact, such as the rotating mandrel described, is 75 such that it is not necessary to shift this contact continuously, although, of course, continuous shifting or rotating of the mandrel is desirable.

While there are a number of liquids suitable for dipping the coils of wire, I prefer to use the following:

|                       | Parts by weight |
|-----------------------|-----------------|
| China wood oil        | 30              |
| Glycerine ester rosin | 20              |
| Petroleum naphtha     | 50              |

The above mixture should be diluted with additional naphtha to give the proper thickness of coating on the finished wire, which thickness varies with the shape, size and exact use to which the wire is put. I may also add small quantities, about 1%, of dryers such as litharge, manganese dioxide, etc., as may be desirable to assist the coating in taking its 95 set or losing its tackiness quickly while drying. Heat and/or moving air also assists in drying and usually produces a harder, smoother coating.

Also I prefer to add a pigment, such as 100

ultra-marine blue, because the coating is transparent and does not permit ready identification in the wire mill in which the wire is made or in the users' hands.

5 Still another mixture is as follows:

|                   | Parts by weight |
|-------------------|-----------------|
| Rosin             | 15.0            |
| Hydrated lime     | 0.9             |
| 10 Litharge       | 0.3             |
| Manganese dioxide | 0.2             |
| China wood oil    | 33.6            |
| Naphtha           | 50.0            |

15 The rosin, salts and oil are cooked to a heavy body and thinned with the naphtha, after which additional naphtha and pigment is added as required. In both of the above formulæ, turpentine or coal tar naphtha may be used as a solvent or dilutent. It will be 20 seen that in both of the mixtures the combined properties of a rosin like substance and a long oil or varnish are provided.

I claim:

1. The method of coating a wire, which 25 consists in applying to the wire in coil form the coating material in a liquid form, and drying the wire while suspended on a rotating support upon which it is constantly changing its position thereon.

30 2. The method of cement coating a wire, which consists in applying to a coil of the wire the cementing material in liquid form, extending the coil, placing the extended coil loosely upon a support and rotating the support.

35 3. The method of cement coating a wire, which consists in applying to a coil of the wire the cementing material in liquid form, suspending the coil loosely upon a rotating 40 support positioned within the coil, and drying the coil.

4. The method of cement coating a wire, which consists of applying to a coil of the wire the cementing material in liquid form, 45 extending the coil, suspending it loosely upon a support positioned within the coil, rotating the support and drying the coil.

5. The method of cement coating a wire, which consists in dipping the wire in a coil in a liquid cementing material, extending it, placing it upon a support, drying the coil and shifting the support relatively to the coil during the drying operation.

6. The method of coating a wire, which 55 consists in applying the coating material as a liquid to the wire, placing the wire upon a support, solidifying the material on the surface of the wire, and continuously shifting the support with respect to the wire during 60 the solidification operation.

7. The method of coating a wire, which consists in applying to the surface thereof materials having the gumminess of rosin, and the flexibility of a long oil or varnish, placing the wire upon a support, and constantly

changing the position of the wire upon the support during the time such materials are solidifying on the surface, whereby to obtain a smooth and uniformly distributed coating.

8. The method of cement coating automatic stapling machine wire, which consists in dipping a coil of the wire in a mixture of China wood oil, glycerine ester gum and petroleum naphtha, and extending the coil on a contact support and rotating such support so as to give a shifting contact during the drying of the mixture, thereby obtaining on the surface of the wire a comparatively smooth coating rendering the wire suitable for automatic staple forming and driving machines.

In testimony whereof I have hereunto subscribed my name.

J BIRCHARD GREEN.

70

75

80

85

90

95

100

105

110

115

120

125

130